

Patented Sept. 3, 1935

2,013,185

# UNITED STATES PATENT OFFICE

2,013,185

## COATING FOR VESSELS

Ross C. Powell, Forest Hills, N. Y., assignor to  
The Texas Company, New York, N. Y., a corporation of Delaware

No Drawing. Application June 24, 1932,  
Serial No. 619,127

### 2 Claims. (Cl. 91—70.1)

This invention relates in general to corrosive resistant vessels and more especially to a method of coating a vessel with a corrosive resistant material.

5 In many operations involving the use of vessels subjected to high temperatures and in some instances high pressures, and where a corrosive substance is being treated, it is generally the practice to fabricate these vessels to a thickness 5 sufficiently great to provide for future corrosion without sacrificing safety. Iron or carbon steel, due to its cheapness and strength is generally employed. These metals are readily attacked by corrosive substances and, for example, in the treatment of hydrocarbon oils the free sulphur and/or sulphur compounds evolved during the treatment rapidly corrode the portions of the vessel with which they contact.

10 It is of prime importance in the coating of a vessel with a corrosive resistant material to provide a surface of a non-porous nature which is impervious to corrosive substances. If the coating is porous, which presents what is commonly known as pits in the coating surface, the corrosive substance being treated, whether in liquid or vaporous form, enters these pits and attacks the base metal. The deleterious effects of spotted corrosion are not only hard to detect but also 15 greatly impair the safe operation of the vessel.

20 In the treatment of hydrocarbon oils in a pressure still or vessel, the vapors or liquid enter the pits and gradually corrode the base metal to such an extent that future operation of the same would be extremely dangerous. It would 25 be advantageous, therefore, to provide a coating on the inside shell of a metallic vessel free from pits and capable of resisting corrosion.

25 In accordance with my invention there is provided a method of applying a corrosive resistant metal or metal alloy coating to the interior of a vessel which closely adheres to the base metal and presents an even smooth surface characterized by the lack of porosity or pits extending through to the base metal.

30 An object of my invention is to provide a method of coating the interior of a vessel with a corrosive resistant coating of a homogeneous nature and free from pits.

35 Another object of my invention is to provide a method of coating the interior of a vessel by spraying a corrosive resistant metal or metal alloy therein while the vessel is at an elevated temperature.

40 A further object of my invention is to provide a method of coating the interior of a vessel by

spraying a corrosive resistant metal or metal alloy therein while the vessel is at an elevated temperature and being rolled.

45 Still another object of my invention is to provide a vessel having a corrosive resisting coating applied thereto while the vessel is being rolled and at a high temperature.

50 With these and other objects in view, which may be incident to my improvement, the invention consists in the several method steps to be 5 hereinafter set forth in detail for providing an interior coating for a vessel, with the understanding that the several steps may be varied without departing from the spirit and scope of the appended claims.

55 My invention may be carried out with a vessel of any size or shape. While it will be described in connection with large vessels, it is equally applicable to smaller ones, such for instance, as tubes forming a heating coil for use in the conversion of hydrocarbon oils.

60 A large vessel may be made from a single billet of metal, such as carbon steel. The billet may be of the pierced billet type and forced to the desired size and shape by a plurality of rollers suitably positioned with respect to the pierced billet. A vessel may also be made up of a plurality of sections. The sections to be formed into the vessel are rolled to the correct curvature and spot welded together at the joints. The joints are 65 then grooved out and further welded by special welding machines to form tight joints.

70 In accordance with my invention an interior coating of corrosive resistant material is applied to any type vessel to prevent corrosion of the base metal. The corrosive resistant material may, for instance, be chromium or one of its alloys. It is well known that chromium or its alloys possess high corrosive resistant properties, especially to the corrosive substance present or evolved 75 in the cracking of hydrocarbon oils. Another metal possessing high corrosive resistant properties is aluminum and this metal can also be used as a coating as will hereinafter appear.

75 My invention will now be described in connection with coating the interior of a vessel manufactured by either of the above mentioned methods with a corrosive resistant material, although it is to be clearly understood that the invention is applicable to a vessel manufactured by any 80 method, whether new or previously used.

85 In manufacturing a vessel with a single billet of the pierced type, the billet is rotated while at an elevated temperature and this rotation with the aid of suitable rollers forms a vessel of the 85

desired size and shape. When the vessel has reached the desired size and shape, it is still at an elevated temperature and is allowed to gradually cool. My invention has to do with the application of the corrosive resistant coating while the vessel is still at an elevated temperature and being rotated.

I propose to insert a "Schoop" gun or any other suitable type of pressure spraying device 10 into the interior of the vessel. The spraying device is adapted to spray the corrosive resistant material in a molten state evenly onto the interior surface of the vessel with great force and while the vessel is still at an elevated temperature. 15 Prior to the spraying of the interior of the vessel, it has been found desirable to remove the scale which has been formed thereon. This may be accomplished by inserting superheated steam under pressure into the vessel which functions 20 to remove the scaling particles. While I have mentioned steam as being satisfactory for removing the scale, it is to be understood that other scale removing mediums, may be employed. It is also within the scope of my invention to use a 25 flux, whether a scaling medium has been used, or not, to aid fusion between the coating material and the base metal.

After the scale has been removed and the vessel is still at an elevated temperature, the molten 30 corrosive resistant material is forced through the spraying device at a plurality of outlets. This material contacts the interior of the vessel with great force and due to the elevated temperature of both the vessel and the corrosive resistant material, fusion between the two takes place. The 35 chromium coating not only forms a layer above the base metal but also penetrates same and alloys therewith to form in effect an integral surface coating. Another feature of my invention 40 is the application of the coating material while the vessel is being rolled. I have found that the rolling operation aids in the fusion of the coating material with the base metal and reduces the porosity thereof. Moreover, the rolling operation 45 tends to even out the coating material and provides a smooth homogeneous coating of uniform thickness throughout.

In providing a chromium coating in accordance with my invention, the billet is heated to a 50 temperature of around 2400° F. and rolled at this temperature on suitable rollers to form a vessel of the desired size and shape. Superheated steam or any other suitable scaling medium is then introduced into the rotating vessel to remove any scale formed on the interior thereof. 55 The temperature of the vessel is then reduced to between 1900° and 2300° F. and the chromium coating in a molten form is evenly sprayed onto the interior of the vessel by the pressure spraying 60 device. The chromium readily fuses with the base metal of the vessel between these temperatures and this fusion together with the rolling action causes the chromium to penetrate the base metal and closely adhere thereto and form a 65 smooth homogeneous coating free from pits. The thickness of the coating will vary depending upon the quantity of chromium forced through the spraying device. I have found that a coating as thin as 1/100 of an inch is satisfactory in 70 view of the excellent corrosive resistant properties of chromium. While I have specifically mentioned the application of chromium as a coating material, it is to be understood that chromium alloys, such as chromium and nickel and chromium-iron and nickel or any other chromium al-

loys may be used. The thickness of the resisting coating has been merely given as an example and it is to be clearly understood that this thickness may also be varied without departing from the spirit of my invention.

Aluminum is also very satisfactory in resisting corrosion, especially in the treatment of hydrocarbon oils. If an aluminum coating is used, the vessel is cooled to a temperature of say, between 900° to 1150° F. and the rolling operation continued. The aluminum may be applied either in a molten or powdered form to the interior surface, after the scale has been removed, by any suitable pressure device such as a "Schoop" gun. The aluminum readily fuses with the base metal 15 between these temperatures and forms a protective coating free from pits and of a smooth homogeneous nature. As in the case of applying a chromium coating to the interior of the vessel, the rolling of the vessel and the application of the aluminum while the vessel is at an elevated temperature forms in effect an integral surface coating of a non-porous nature.

Aluminum foil may also be used in accordance with my invention. Aluminum foil is available 25 in sheet form and a sheet or the necessary number of sheets of the foil may be inserted into the vessel to properly cover the interior or any desired portion thereof. The heat of the vessel, that is between 900° and 1150° F., is transmitted 30 to the aluminum foil. This transmittal heat starts fusion between the aluminum foil and the base metal of the vessel and this fusion aided by the rolling operation provides an aluminum coating of a smooth homogeneous nature free from 35 pits and capable of resisting corrosion. I propose to use aluminum foil made up in sheets of approximately 1.5/100 of an inch thickness. This specific thickness, however, is merely given as an example as obviously my aluminum coating 40 may be applied in varying degrees of thickness and with one or more layers, if desired.

When a vessel is made in sections and the sections suitably welded together, heat is applied to satisfactorily anneal the various joints. The vessel is generally placed in a suitable furnace for the annealing operation. It is during this operation that I propose to carry out my invention on a vessel manufactured by this method. The vessel during the annealing operation may be raised to a temperature sufficiently high to correctly anneal same and also to present a sufficiently hot interior surface to the coating material to be applied. After the temperature of the vessel has been raised, a protective coating may be applied 50 in the manner already described. The vessel may also be rolled by any suitable means as the protective coating is being applied.

My invention has been primarily described in connection with the manufacture of new vessels. It is to be understood that it is likewise applicable to the coating of the interior of old vessels to prevent further corrosion thereof. In carrying out my invention with an old vessel, the interior thereof may be suitably sand blasted to remove 65 all deposits therefrom. The vessel may then be heated by any suitable heating device and raised to an elevated temperature. Any scale resulting from the heating operation may be removed, and the protective coating applied as already 70 described. If the vessel is in place, corrosive resistant foil in a sheet or sheets may be inserted within the vessel, after same has been cleaned, and the heating and rolling action will cause the coating material to fuse with the base 75

metal to provide a non-porous protective coating of a smooth homogeneous nature.

My protective coating of corrosive resistant material may also be applied to vessels in place by any suitable spraying device. The vessel is first sand blasted to remove any deposits and raised to a high temperature in any suitable manner, such as by suitably firing same. The scale is removed and when the temperature of the vessel has reached the point where the base metal will readily fuse with the coating material, the coating material is sprayed onto the interior surface of the vessel in molten form with great force. By evenly spraying the corrosive resistant material onto the interior of the vessel with great force, the protective layer tightly adheres to and penetrates the base metal to such an extent as to provide a non-porous and smooth homogeneous coating.

The heating operation described herein, whether it be in the manufacture of a new vessel or the application of a coating to an old vessel, may be carried out under ordinary atmospheric conditions or under sub-atmospheric conditions. Moreover, the coating may be applied in the presence of an inert gas, such as nitrogen.

From the foregoing it will be readily seen that I have provided a method whereby a non-porous homogeneous coating of corrosive resistant material is evenly applied to the interior of a vessel. While I have specifically mentioned that my invention is well adapted to prevent the corrosive action of hydrocarbon oils while being treated, it is to be understood that it is not limited to vessels used in such processes as obviously it is ap-

plicable to the treatment of corrosive substances in general.

I wish it to be understood that I do not confine myself to the precise details herein set forth in the preferred manner of carrying out my invention as it is apparent that many changes and variations may be made by those skilled in the art without departing from the spirit of the invention, or exceeding the scope of the appended claims.

I claim:

1. A method of protecting the interior surface of an oil refining vessel from corrosion which comprises heating said vessel to a temperature in the neighborhood of from 1900 to 2300° F., applying a chromium lining to said vessel in finely divided form while said vessel is at said elevated temperature and thereafter applying mechanical pressure to said lining to form a dense, compact coating of substantially uniform thickness. 10 20

2. A method of manufacturing an oil refining vessel having a protective lining which comprises heating a metal billet to a temperature in the neighborhood of 2400° F., thereafter rolling said billet into a vessel of the desired size and shape, 25 thereafter removing scale formed as a result of said rolling operation, spraying chromium in molten form against the interior surface of the vessel so formed and while said vessel is at a temperature ranging from 1900 to 2300° F., and thereafter applying mechanical pressure to said lining to form a dense, compact coating within said vessel. 30

ROSS C. POWELL.